

Patented Sept. 1, 1925.

1,552,201

## UNITED STATES PATENT OFFICE.

JOHANNES J. BERGSMA, OF WELTEVREDEN, JAVA.

## PROCESS FOR PREPARING INCOMBUSTIBLE AND INSULATING MATERIAL.

No Drawing.

Application filed September 15, 1922. Serial No. 588,479.

*To all whom it may concern:*

Be it known that I, JOHANNES J. BERGSMA, a subject of the Queen of the Netherlands, and residing at Weltevreden, Java, Nether-  
5 land East India, have invented certain new and useful Improvements in Processes for Preparing Incombustible and Insulating Materials, of which the following is a specification.

10 This invention relates to a process for preparing incombustible and insulating materials and is based upon the use of the bark of trees, the said bark being mixed with suitable inorganic substances and binding mate-  
15 rial, according to the desired appliances of the materials to be prepared.

Processes for the preparation of plastic materials are also known, in which in a similar way use is made of wood (wood-dust, 20 chips, shavings, etc.) and it is also known to use cork, the bark of the cork-oak, for similar appliances.

According to the present invention use can be made of the bark of all kinds of trees, 25 which material is obtainable in large quantities everywhere and nearly without value. As an example of a bark which has been found suitable for the execution of the process it is pointed at the bark of the djatti 30 tree growing in India, but as a matter of fact the invention is not limited to the employment of that kind of bark, as most of the kinds of trees existing in the world supply a material which is suitable for the practice of the invention.

In the execution of the process according to the invention, the raw bark will preferably be lixiviated in a hot state, thereupon pressed, dried and disintegrated. After ad-  
40 mixture of suitable filling substance or substances, chosen according to the appliances aimed at a binding material is added and the mixture is worked up to a homogeneous pappy or pulpoous mass which can be em-  
45 ployed in several ways. In one form of execution of the invention the mass is moulded to form-pieces of the desired shape in a moulding machine of any known construction, in which the mass is pressed and thereafter the so obtained form-pieces are carried to a drying room for desiccation and can if desired finally be planed or polished at their surface. In another form of execu-  
50 tion of the invention the mass is applied

by way of an insulating layer upon other 55 materials, such as timber or iron.

The following example of the preparation of a plastic mass is given for the sake of more clearly emphasizing the manner where-  
in the claimed process can be carried out. 60

Pulverized bark, Portland cement and in-  
fusorial earth are thoroughly mixed in dry 65 condition in the proportion of 1 : 2 :  $\frac{1}{2}$  parts in weight, and thereupon a sufficient quantity of diluted molasses is added to the 70 mixture, which is worked up so as to obtain a homogeneous pappy mass to be moulded under a relatively light pressure or a wet mass to be applied in a thin layer upon the timber, iron or other construction to 75 insulate.

The above composition can be varied in many respects as for the kind and the proportions of the filling and binding materials used in admixture with bark. 80

E. g. the infusorial earth can in many cases be dispensed with so that the admixture consists only of cement and molasses. Further the more expensive Portland cement can be substituted by brick dust and sand. 85 Also many other filling materials may be taken into account, while molasses may be substituted by other organic binding substances. According to the properties of the matters used in admixture with the bark 90 the final products obtained will be lighter or heavier.

As referred to above the products prepared according to the invention are highly 90 recommendable for insulating any wood metal or other construction and making it incombustible by covering it with a thin superficial layer of the new material. Besides, it has been found of extreme economic 95 importance for all building purposes, such as walls, floors, roofing, etc.

Having now particularly described and ascertained the nature of my said invention and the manner in which it is to be performed what I claim as new and wish to secure by Letters Patent is:

1. A process of preparing an incom-  
bustible and insulating material consisting in mixing pulverized bark of the djatti tree with a binding material. 105

2. A process of preparing an incom-  
bustible and insulating material consisting in mixing pulverized bark of the djatti tree

with a binding material and a filling substance.

3. A process of preparing an incom-  
bustible and insulating material consisting  
in mixing cork-free pulverized bark of trees  
with a filling substance and with a binding  
material including molasses.

4. A process of preparing an incom-

bustible and insulating material consisting  
in mixing cork-free pulverized bark of trees <sup>10</sup>  
with Portland cement, infusorial earth and  
diluted molasses, said bark, cement and in-  
fusorial earth being mixed in the proportion  
of 1:2:1/2 parts in weight.

In testimony whereof I affix my signature.

BERGSMA.